

Oct. 29, 1940.

E. H. VAN SCHOICK

2,219,606

FIREBRICK AND METHOD OF MAKING SAME

Filed March 13, 1939



Inventor:  
Elmer H. Van Schoick

By Davis, Lindsay, Shultz & Shantz  
Atty

## UNITED STATES PATENT OFFICE

2,219,606

FIREBRICK AND METHOD OF MAKING  
SAMEElmer H. Van Schoick, Ottawa, Ill., assignor to  
Chicago Retort & Fire Brick Company, Chi-  
cago, Ill., a corporation of Illinois

Application March 13, 1939, Serial No. 261,467

9 Claims. (CL 25—156)

My invention relates to fire brick and to the method of making the same, and is more particularly concerned with brick of the stiff mud process type that is characterized by a low spalling loss in service.

Spalling is the term applied to the chipping, crumbling, or falling away of the brick at the exposed surface which is directly subjected to the heat of the furnace and which attains a considerably higher temperature than the opposite surface. A sharp temperature gradient, therefore, exists across each brick which is reflected after a period of service by very definite changes in the brick and these changes have long been recognized as a major cause of failure in refractories. Primarily, spalling is due to the changes which occur in the directly heated layer of brick.

It has been ascertained that a new clay brick furnace wall has a relatively high degree of initial resistance to thermal spalling, but this resistance is not maintained throughout the life of the refractory. Generally speaking, the loss in resistance to spalling is due to the creation of a vitrified layer extending inwardly from the exposed face of the brick for a distance of from  $\frac{1}{2}$  inch to  $1\frac{1}{2}$  inches, and also to volume changes in the vitrified layer, relative to the original volume of this portion of the brick, which sets up stresses that may be increased by subsequent thermal changes to a point where portions of the vitrified layer crack and "spall off." A further factor in spalling is the contaminating action of slag.

Spalling is a particular problem in bricks made by the stiff mud process because of a condition inherent in the method of manufacture. In this process, the clay is extruded through a tapered die to form a stiff mud column which is then cut transversely to form brick blanks. If standard straights having dimensions of  $9'' \times 4\frac{1}{2}'' \times 2\frac{1}{2}''$  are to be made from the blanks, the cutting of the column establishes the thickness dimension of the brick with allowance for final compression and shrinkage due to drying and burning, while the cut surfaces, or the cross-section of the column, form the larger or  $9'' \times 4\frac{1}{2}''$  faces of the brick. Pressure is then applied to the two larger surfaces of the blank thus formed to produce the finished brick.

Due to the extrusion of the clay through the tapered die, the core of the column moves at a faster rate through the die than the outer portions thereof and this action produces characteristic and so-called flow lines which are readily apparent in the finished brick and extend generally lengthwise of the clay column. Generally speak-

ing, these flow lines form a concentric pattern around the longitudinal axis of the clay column and, accordingly, of the corresponding axis portion in the finished brick which is normal to the large faces thereof. This pattern may be diagrammatically illustrated as a succession of concentric circles, or other shaped enclosures depending upon the shape of the die and its extrusion opening, extending from the column axis to the external surfaces of the column. After the brick has been burned, these flow lines become what might be termed "planes of cleavage" so that when laid to form a furnace wall with its  $9'' \times 2\frac{1}{2}''$  face exposed to the heat, it is apparent that the disposition of the flow lines, i. e., generally parallel or located at a slight angle to the exposed face of the brick, favors, when spalling does occur, the crumbling and falling away of large portions of the exposed face, thus reducing the working thickness of the brick.

It is therefore, the principal object of my invention to devise a fire brick which materially reduces the aforesaid spalling loss, although made from a clay column extruded by the stiff mud process, and to a method of manufacturing this brick.

These and further objects of my invention will be set forth in the following specification, reference being had to the accompanying drawing, and the novel means by which said objects are effected, will be definitely pointed out in the claims.

In the drawing:

Figure 1 is a diagrammatic, elevational view of a typical brick-blank forming machine, as commonly used in the manufacture of bricks made by the stiff mud process.

Figure 2 is a perspective view of a typical fire brick made by the stiff mud process and showing the relation of the flow lines to the larger faces thereof.

Fig. 3 is a perspective view of a brick similar to that shown in Fig. 2, after the brick has undergone a period of service in an industrial furnace and showing the characteristic spalling due to the relation of the flow lines in the brick to the exposed face thereof.

Fig. 4 is a perspective view of a brick blank, as severed from the clay column illustrated in Fig. 1, and showing the characteristic flow line pattern around that axis of the blank which coincided with the longitudinal axis of the column.

Fig. 5 is a perspective view of a brick formed by applying pressure to the top and bottom surfaces of the blank illustrated in Fig. 4, and showing the flattened and generally deformed appearance

5

10

15

20

25

30

35

40

45

50

55

which the flow line pattern presents in the finished brick, particularly with reference to the exposed surface thereof.

For convenience, the invention will be described in connection with the manufacture of a standard straight fire brick having dimensions of 9" x 4 1/2" x 2 1/2", although it will be understood that the invention is capable of application to the manufacture of fire brick having different dimensions.

Referring to Fig. 1 of the drawing, the numeral 10 designates a typical brick-blank forming machine which is loaded with the desired type of fire clay that is extruded by means of an auger 15 or screw 11 through a tapered die 12 to form a clay column 13 that is ordinarily deposited on an endless conveyor and moved away from the die at a rate equal to its speed of extrusion. After the column has moved a convenient distance from the die, it is periodically cut by a plurality of spaced wires in the usual manner to form a plurality of brick blanks 14. For purpose of illustration, it will be assumed that the thickness of the column 13, as viewed in Fig. 1, corresponds to the 4 1/2 inch dimension of the finished brick and that the spacing of the cutting wires is such as will provide the desired thickness of 2 1/2 inches in the finished brick.

For reasons already noted, this manner of producing the clay column creates flow lines which extend longitudinally thereof and, therefore, generally normal to the wire cut surfaces of the blank 14. In the present manufacture of fire brick from this type of column, each blank 14 is 30 rested on one of its larger surfaces, i. e., rotated through an angle of ninety degrees from the position illustrated in Fig. 1, and the blank is then compressed between its large faces, or in a direction generally parallel to that axis of the blank 35 which originally coincided with the longitudinal axis of the column.

The fire brick thus produced is illustrated in Fig. 2 and it will be particularly noted that the flow lines, indicated by the numeral 15, are generally parallel to the 9" x 2 1/2" face 16 of the brick 40 which ordinarily constitutes the exposed face of the brick in furnace operations.

In Fig. 3 is illustrated the brick shown in Fig. 2 after it has undergone a period of duty in a furnace and the numeral 17 indicates generally the roughened surface of the brick occasioned by spalling of the exposed face 16 and which occurs 45 generally along the flow lines 15.

I have ascertained that it is possible to make fire brick by the stiff mud process and to take advantage of the characteristic flow lines created in the clay column as a means of materially reducing the spalling loss in fire brick made therefrom. Generally speaking, the improvement consists in so arranging the flow lines with reference 50 to the exposed face of the brick that if spalling does occur, the spalled portions of the brick which would otherwise fall completely away from the brick, or be readily loosened during the operation of lancing, or by the insertion of other types of bars in the furnace, will remain in place and may 55 in fact, due to the displacement of the flow line pattern, as hereinafter described, be substantially interlocked with other portions of the brick. The 60 integrity of the exposed face of the brick is therefore maintained for a considerably longer time 65 than is possible with the brick construction illustrated in Fig. 2.

In making my improved brick, each brick blank 14 is compressed between its top and bottom surfaces, as viewed in Fig. 1, and as diagrammatically

illustrated in perspective in Fig. 4, that is, pressure is applied to a pair of the opposite faces of the brick normal to that axis of the brick which coincided with the longitudinal axis of the clay column 13. This method does not require a change in position of the brick, as is necessary in the making of the brick illustrated in Fig. 2, and the final results of the compression are illustrated in the brick shown in Fig. 5. The 9" x 4 1/2" face 18 of the brick blank shown in Fig. 10 4 has been compressed to form the 9" x 2 1/2" exposed face 19 in which the flow line pattern has been generally compressed and deformed to the extent diagrammatically illustrated in Fig. 5. The original 9" x 2 1/2" and 2 1/2" x 4 1/2" faces 15 of the blank are transformed by the compression into the 9" x 4 1/2" and 4 1/2" x 2 1/2" faces, respectively, of the brick, the length of the blank being unchanged by the compression.

It will be particularly noted that the flow lines 20 in this brick are normal to and extend from the exposed face of the brick into the body thereof. Accordingly, if cracking of this face does occur when exposed to the usual temperatures, it will generally progress along the planes of cleavage 25 established by the flow lines, as in the type of brick illustrated in Fig. 2, but due to the flow line relation to the exposed face, the cracked pieces are more likely to rest in their original positions than is possible with the brick shown in Fig. 2 30 where the flow lines are parallel to the exposed face.

Moreover, the compressing of the brick blank in Fig. 4 not only flattens the flow line pattern, but effects some deformation thereof and a lateral 35 flow of the mud which results in an interlocking of fragments of the brick along the flow lines in the heated layer of the brick and this condition also acts to reduce the spalling loss.

The advantages of my improved brick can be 40 better understood by a comparison of the results obtained in a panel spalling test of the bricks illustrated in Figs. 2 and 5. This test was developed by the American Refractories Institute as a means of determining the spalling behavior 45 of fire brick in service and the test has been adopted by the American Society of Testing Materials.

Briefly, the principle of this spalling method is to test a section of a furnace wall rather than 50 individual bricks and in carrying out the method, fourteen bricks are formed in a wall panel, corresponding to a section of the wall of an industrial furnace, the panel being eighteen inches square and each brick having its 9" x 2 1/2" face 55 exposed for treatment. This panel surface is then heated to 1600° C. (2912° F.) for a period of twenty-four hours and the back of the panel is insulated to maintain a temperature of about 1250° C. on the cool side of the brick. The object 60 of this preheating is to develop in the brick those changes which occur after longer periods of operation at the lower temperatures encountered in industrial practice and, in particular, a vitrified layer along the heated face of the brick that generally corresponds to the layer produced under 65 actual working conditions.

Having thus conditioned the panel, it is then tested for thermal spalling by heating to a temperature of 1400° C. (2552° F.) for a period of ten minutes and then rapidly cooling for ten minutes by exposing the panel to an air water blast, after which the panel is again heated for a period of ten minutes and this alternate heating and cooling is continued for twelve complete cycles, each cycle requiring twenty minutes.

The panel is then dismantled and from each brick is removed those pieces that separate easily, but no attempt is made to remove pieces that require prying or tapping. The percentage loss in weight as determined by this test indicates the spalling resistance of the brick for a given class of service.

The type of fire brick illustrated in Fig. 2, when subjected to the foregoing test, has shown as much as a twenty per cent loss in weight from spalling, as compared to a loss of five per cent or less for the brick illustrated in Fig. 5.

It has been ascertained that due to the relation of the flow lines to the exposed face of my improved brick, the latter is characterized by an increased resistance to abrasion, whether of a solid, liquid, or gaseous nature. When the exposed faces of the fire bricks illustrated in Figs. 2 and 5 are held against a grinding wheel, it has been determined that the grinding of the face in the Fig. 2 type of brick can be accomplished with considerably more ease than in the Fig. 5 type of brick, and this condition is believed to be due to what might be termed the "grain" of the respective bricks as established by their flow lines. In the Fig. 5 type of brick, for example, the pressure of the grinding wheel is "across the grain" as compared to the grinding "with the grain" in the Fig. 2 type of brick.

The practice of my invention is not restricted to disposing the flow lines normal to the 9" x 2½" face of a standard straight, since these lines may be similarly related to the end or 4½" x 2½" face of the same type of brick, or to any comparable faces of other style of brick. For example, in straights intended for header courses, the mud column could be extruded through a die measuring 4½" x 2½", cut off at intervals of 9 inches, and then compressed between its 9" x 2½" faces to a thickness of 2½ inches and a width of 4½ inches.

A further method of making the bricks and still accomplishing a disposition of the flow line pattern normal to the exposed face of the brick can be secured in the case of a brick having a 9" x 2½" exposed face by extruding the clay through a die having similar dimensions. In this case, then, the flow lines, as before, will extend generally parallel to the longitudinal axis of the extruded clay column, but due to the manner of extrusion, the flow lines are already normal to a transverse plane through the column. Accordingly, when this column is cut at 4½" intervals to form a brick length, it is simply necessary to compress this blank between its 9" x 2½" faces. This method, however, does not secure a deformation of the flow line pattern, as illustrated in Fig. 5. A brick of this character can be employed for stretcher courses in the same manner as the bricks illustrated in Fig. 5.

In the case of header courses, that is, where the exposed faces of the brick are constituted by the 4½" x 2½" face, the brick may be formed by extruding the clay column through a forming die having similar dimensions and then cutting the column at 9" intervals. This brick then would be compressed between its 4½" x 2½" faces to fully form the brick for burning.

I claim:

1. The method of making stiff mud, fire brick which comprises extruding under pressure a stiff mud column through the tapered discharge opening of a brick machine, the extrusion creating flow lines extending throughout the length of and generally parallel to the longitudinal axis of the

column, severing the column transverse to the axis to form a brick blank in which the flow lines are normal to the severed faces, and then compressing the blank between a pair of its opposite faces other than the severed faces sufficient to cause a pronounced lateral flow of the mud composing the blank and a substantial decrease in the dimension of the blank in the direction of the applied pressure and thereby provide a brick in which a deformed severed face constitutes the face of the brick which is exposed to the heat, the flow lines being normal to the exposed face and the compression and lateral flow tending to create interlocking pieces of the brick in that layer of the exposed face which becomes vitrified during service.

2. The method of making stiff mud, fire brick which comprises extruding under pressure a stiff mud column through the tapered discharge opening of a brick machine, the extrusion creating flow lines extending throughout the length of and generally parallel to the longitudinal axis of the column and the column having a rectangular cross section whose area approximates that of one of the largest faces of the brick, severing the column transverse to the axis to form a brick blank in which the flow lines are normal to the severed faces, and then compressing the blank between a pair of its opposite faces other than the severed faces sufficient to cause a pronounced lateral flow of the mud composing the blank and a substantial decrease in the dimension of the blank in the direction of the applied pressure while maintaining the other dimension of the severed faces and thereby provide a brick in which a deformed severed face constitutes the face of the brick which is exposed to the heat, the flow lines being normal to the exposed face and the compression and lateral flow tending to create interlocking pieces of the brick in that layer of the exposed face which becomes vitrified during service.

3. The method of making stiff mud, fire brick which comprises cutting a stiff mud brick blank from a stiff mud column having flow lines extending throughout the length of and formed by pressure extrusion of the column through the tapered discharge opening of a brick machine, the flow lines extending throughout the body of the blank and generally normal to the cut faces, and then compressing the blank between a pair of its opposite faces other than the cut faces sufficient to cause a pronounced lateral flow of the mud composing the blank and a substantial decrease in the dimension of the blank in the direction of the applied pressure and thereby provide a brick in which a deformed cut face constitutes the face of the brick which is exposed to the heat, the flow lines being normal to the exposed face and the deformation and lateral flow tending to create interlocking pieces of the brick in that layer of the exposed face which becomes vitrified during service.

4. A fire brick made in accordance with the method defined in claim 1.

5. A fire brick made in accordance with the method defined in claim 2.

6. A fire brick made in accordance with the method defined in claim 3.

7. A fire brick of the stiff mud process type having flow lines created by pressure extrusion through the tapered discharge opening of a brick machine extending through the body of the brick normal to that face which is exposed to the heat and becomes vitrified during service, the lines

forming a grain-like pattern pressure disarranged relative to the original extrusion pattern sufficient to cause a pronounced flow of mud along the flow lines and creating interlocking pieces of brick 5 in the vitrified layer which substantially enhances its resistance to spalling and erosion.

8. A standard straight first brick of the stiff mud process type having flow lines created by pressure extrusion through the tapered discharge 10 opening of a brick machine, extending through the body of the brick normal to that 9" x 2½" face which is exposed to the heat and becomes vitrified in service, the lines forming a grain-like pattern pressure disarranged relative to the original 15 extrusion pattern sufficient to cause a pronounced flow of the mud along the flow lines and creating interlocking pieces of brick in the vitri-

fied layer which materially enhances its resistance to spalling and erosion.

9. A standard straight fire brick of the stiff mud process type having flow lines created by pressure extrusion through the tapered discharge 5 opening of the brick machine, extending through the body of the brick normal to that 4½" x 2½" face which is exposed to the heat and becomes vitrified during service, the lines forming a grain-like pattern pressure disarranged relative to the original 10 extrusion pattern sufficient to cause a pronounced flow of the mud along the flow lines and creating interlocking pieces of brick in the vitrified layer which substantially enhances its resistance to spalling and erosion. 15

ELMER H. VAN SCHOICK.